

No. 863,293.

PATENTED AUG. 13, 1907.

H. W. LEONARD.  
ELECTRIC RESISTANCE DEVICE.  
APPLICATION FILED MAR. 21, 1905.

*Fig. 1*



*Fig. 7*



*Fig. 4*



*Fig. 5*



*Fig. 6*

H. Ward Leonard

Witnesses

S. R. Dager.  
Geo. A. Hoffman.

Inventor

By his Attorney C. W. Edwards.

# UNITED STATES PATENT OFFICE.

HARRY WARD LEONARD, OF BRONXVILLE, NEW YORK.

## ELECTRIC RESISTANCE DEVICE.

No. 863,293.

Specification of Letters Patent.

Patented Aug. 13, 1907.

Application filed March 21, 1905. Serial No. 251,231.

*To all whom it may concern:*

Be it known that I, HARRY WARD LEONARD, a citizen of the United States, residing at Bronxville, in the county of Westchester and State of New York, have 5 invented certain new and useful Improvements in Electric Resistance Devices, of which the following is a full, clear, and exact specification.

My invention relates to resistance devices and particularly to the method and means for supporting, protecting, insulating, and mechanically, electrically and chemically improving resistance devices, such as rheostats, electric heaters, etc., and the essential object of 10 my invention is to produce improvement as above stated.

15 One of the applications of my invention is in the manufacture of resistance units relative to which I will now describe my invention.

In making resistance units I prefer to employ a tubular support made of fictile material such as porcelain.

20 The coefficient of heat dilatation of such material is quite low relative to that of metals such as I prefer to employ for the resistive conductor. For many well known reasons I prefer to use a metallic conductor embedded in a coating of adhesive material on the surface

25 of the support. Heretofore when the resistive conductor, the support and the adhesive attaching coating are heated to a high degree in the process of manufacture the difference between the dilatation of the resistive conductor, the support, and the adhesive attach-

30 ing coating, tend to impair the perfection of the said coating. One way of practically overcoming this difficulty for many forms of apparatus is described in my Patent No. 691949, granted Jan. 28, 1902. In that patent I describe a low fusing vitreous coating which

35 fuses and forms the adhesive attaching coating at a temperature so low that the difference in the dilatations mentioned are not enough to interfere with the commercial production of the desired article. But in many instances resistances are desired which must

40 withstand a development of heat such that the low fusing vitreous coating of the said patent would melt and flow, thereby exposing the resistive conductor, and displacing it, and in some instances causing the low fusing vitreous material to collect into a thick layer on

45 the lower side and even to cause molten drops to fall off in some cases.

It is desirable to employ a material for the adhesive, attaching coating which has a very high fusing point, so that at the heat of practical operations it will not

50 become sufficiently fluid to flow materially. In accordance with my present invention I employ an infusible material for the coating or protective composition in which the conductor is embedded or partially em-

55 bedded and I overcome the difficulties due to dilatation so that the parts are not affected to an objectionable degree by the high temperatures desirable in practice. In instances where I use an adhesive coating for

attaching the resistive conductor to a support of different material from the coating, I prefer to use for this coating a material whose coefficient of expansion by 60 heat is between that of the support and that of the resistive conductor.

I also prefer to use the resistive conductor in a form such as the reflexed form so that the strain in the coating will be reduced. When the conductor becomes so 65 large as to produce detrimental strains in the coating, I prefer to sub-divide the conductor into several smaller conductors and in most cases prefer to braid together the plurality of smaller conductors, or in some equivalent way obtain the total cross section desired while 70 avoiding the objections incidental to having a single practically straight conductor of round cross section embedded in the coating. Sometimes I use a flat metallic tape having such perforations or equivalent openings as to enable the coating to fill in such openings 75 and thereby more firmly attach the resistive conductor.

I prefer to apply the material of the coating to the support and resistive conductor while cold and then form the coating by heating in a muffle furnace or other suitable source of heat external to the resistance. In 80 some cases however, I form the coating by developing all or a part of the heat needed by passing an electric current through the resistive conductor so as to develop in the conductor itself the heat desired. The material of the coating I sometimes apply as a slip; 85 sometimes I apply it as a dry powder, sometimes as a paste, but in all cases I prefer to have such solid material as is employed, in a finely divided state, such as results, for example, from grinding. In some instances the coating or the protective composition need 90 not be highly heated during the process of manufacture, a mere drying or baking being all that is needed sometimes. In many instances I prefer to glaze the coating so as to make the article more waterproof, better as regards insulation, heat and light reflecting, and 95 securing the many well known advantages of a thin glaze on the surface of such a coating. I generally apply two or more coats of the adhesive attaching coating and sometimes form the coating by repeated local applications of the material, but I may in some cases 100 have but a single coating, or layer.

I prefer to always have in the protective composition which is in contact with the resistive conductor a certain material whose coefficient of expansion is higher than that of the resistive conductor and another 105 that is lower, so that by using a suitable proportion of the material of high and low coefficient of expansion, I can obtain the desired coefficient for the protective composition. I prefer to form the protective composition so that as a whole it will not flow at a 110 temperature below 1500° F., and is preferably formed of material which is infusible at the heat of manufacture and has combined with this only a sufficient amount of vitreous material to act as a binder. That

is, the amount of fusible material is so low that the composition as a whole will not be fused sufficiently to flow or assume a glazed appearance.

The following ingredients may be employed to form the composition: ground flint, ground vitreous material and fluorspar. I employ fluorspar because of its high coefficient of expansion. Cryolite may be in some instances substituted for the fluorspar or any similar material which is an equivalent for the purpose of increasing the coefficient of expansion of the coating, or such materials may be combined, for example, I may use both fluorspar and cryolite. It will be noted that both fluorspar and cryolite contain fluorin in combination. I prefer to have a certain amount of boron in the vitreous material. The composition described is tough, coherent, infusible as defined herein, insulating, adhesively attaching to a support, and is protective mechanically and chemically. Moreover, its coefficient of expansion is well suited for use with a resistive conductor having a high coefficient of expansion, and I prefer to use such a conductor on account of the low temperature coefficient which may be secured. While the binding portion of the coating or composition is in many instances not entirely insoluble, yet it is difficultly soluble by comparison with borax, soda, saltpeter and other similar soluble salts which are often employed principally as fluxes, in the manufacture of vitreous enamels. Therefore when I use the term "insoluble" in the claims, I mean substantially insoluble and use the term to exclude what are generally known as soluble salts, rather than to indicate complete insolubility.

In the accompanying drawings, Figure 1 is a side view of one form of my invention; Fig. 2 is a sectional view of one end of the construction shown in Fig. 1 enlarged; Fig. 3 is an enlarged sectional view showing an additional outer coating; Fig. 4 is a plan view of a modification; Fig. 5 is a sectional view on the line 5-5 of Fig. 4; Fig. 6 is a sectional view showing a modification; Fig. 7 is a side view of a modification.

One suitable composition for forming the protective composition or coating contains essentially:—three parts of fluorspar ground to about sixty mesh and four parts of a vitreous material made by fusing together two parts of red lead, two parts of borax and one part of flint, the said vitreous material being ground to a fine powder. The fluorspar of said composition has a coefficient of expansion higher than that of cast-iron and higher than the coefficient of expansion of a resistive conductor made from an alloy of substantially sixty parts of copper and forty parts of nickel. The vitreous material of said composition has a coefficient of expansion less than that of cast-iron or of the said copper-nickel alloy. The composition as a whole has a coefficient of expansion between that of a cast-iron support and the said resistive alloy. When the ground fluorspar is examined under a microscope, the characteristic crystalline form and reflecting surface of the fluorspar crystal is readily observable and can be easily identified when again seen under the microscope. Such a microscopic examination of the protective composition after it is formed by heat, clearly discloses the fact that a large part and perhaps all of the fluorspar remains in its crystalline state and is not so fused as to eliminate the characteristic reflecting, crystalline sur-

face above referred to; that is, the fluorspar in its native state is practically embedded in a matrix of material, which latter material has been sufficiently fused to cause it to form with the fluorspar, a coherent composition adapted to adhere to a suitable support when properly applied and heated in the manner well known to those skilled in the art.

Referring to Figs. 1 and 2, the support is indicated at 1 and is shown as tubular. This support is preferably of some mineral insulating material such as porcelain, 75 glass, terracotta, steatite, lava, various stones, asbestos, mica, or other similar material natural or artificial or both mixed. There are many instances in which the support will be metallic and in that case the coating will be of sufficient thickness to insure good insulation 80 of the conductor from the metallic support. The resistive conductor is indicated at 2 and is shown in the form of a flat braid of wire having an open mesh and as more particularly described in my Patent No. 787,047, granted April 11, 1905. The conductor is embedded 85 in the infusible coating 3 which I have above described and is wound around the support. The conductor is united at the ends to braided terminal leads 4 which are seated in grooves 5 formed in the support and which terminal leads, where they encircle the support, are 90 likewise embedded in the coating.

In Fig. 3 which shows a sectional view of a portion of a resistance unit, there is shown in addition to the infusible coating in which the conductor is embedded, a coating 6 of vitreous material such as glass enamel, and 95 I thereby secure the advantages of a glazed surface as above referred to.

In Figs. 4 and 5 I have shown a support in the form of a plate 7 which may be of iron, or other suitable material. The conductor 8 is shown as reflexed and connected to 100 the terminal contacts 9, the conductor and portions of the terminal contacts being embedded in the infusible coating 3. In some cases the conductor may be only partially embedded, for example, as shown in Fig. 6, in which the conductor 10 is in the form of a reflexed 105 ribbon, having one edge embedded in the insulating material. In some cases this resistive conductor will not itself be embedded in the coating, but will have its terminals or supports embedded or partially embedded in the coating. In some cases the coating itself may 110 form the only support in the finished article. That is, the coating or protective composition may be formed about the conductor so as to form a support in itself, or a temporary support may be employed during manufacture which will not be present in the finished article. 115

In Fig. 7 I have indicated a spirally formed conductor 11 for which there is no other support than the coating or protective composition 3, being somewhat similar to the construction shown in Figs. 1 and 2 except there is no supporting tube. The unit, as shown, is provided with rigid supporting terminals 12 which are fixed to the base plate 13.

It will be understood that various other forms of construction may be developed which will be within the scope of my invention.

Whenever I use the word "powdered" in the claims I mean to describe a material in a finely divided state whether it be dry, or mixed with a fluid so as to be paste-like or cement-like, or whether it be suspended in a liquid so as to be paint-like. Whenever I use the 130

word "infusible" in the claims I mean to describe a material which when subjected to the heat under consideration does not become soft or viscous as a whole, or form a glazed appearance although certain ingredients 5 therein, when considered separately, may become more or less soft or viscous. The material is such that it retains a dull, pottery like surface after being subjected to a visible-red heat. Whenever I use the words "vitreous material" in the claims I mean to describe a 10 material which has been melted by heat to form a material resembling glass for the purposes hereof. By the term "embedding" as used in the claims, I mean either wholly or partially surrounding the conductor and with or without an additional support. Whenever I use the 15 word "glazed" I mean to describe a polished insulating surface impervious to moisture.

Having thus described my invention, I declare that what I claim as new and desire to secure by Letters Patent, is,—

- 20 1. The combination of a resistive conductor, and an infusible composition embedding the conductor, said composition containing fluorin and containing only insoluble materials as essential ingredients when applied to the conductor.
- 25 2. The combination of a resistive conductor, and an infusible composition embedding the conductor, said composition containing fluorspar and containing only insoluble materials as essential ingredients when applied to the conductor.
- 30 3. The combination of a resistive conductor, and an infusible composition embedding the conductor, said composition containing fluorin and boron and containing only insoluble materials as essential ingredients when applied to the conductor.
- 35 4. The combination of a resistive conductor, and an insulating heat resisting composition about said conductor, said composition containing fluorspar in its native state but finely divided and disseminated through the composition and containing only insoluble materials as essential 40 ingredients when applied to the conductor.
5. The combination of a resistive conductor, and a layer of insulating material adhesively attached thereto, said insulating material containing finely divided fluorspar and a binding material, whereby an adhesive layer is produced.
- 45 6. The combination of a support, a resistive conductor, and an insulating coating embedding said conductor, said coating being cohesive and adhesive to the support, infusible, and containing an ingredient whose coefficient of expansion is higher than that of said conductor.
- 50 7. The combination of a resistive conductor, and a coating embedding and protecting said conductor, said coating being coherent and insulating and formed of material part of which is infusible at the heat of manufacture and part of which is fusible, the proportion of fusible material being so low that the coating as a whole is infusible, and said coating containing an ingredient whose coefficient of expansion is higher than that of said conductor.
8. The combination of a resistive conductor, and a solid insulating material embedding said conductor, said material being composed of one ingredient having a coefficient of expansion higher than that of the conductor and another which has a coefficient of expansion less than that of the conductor, one of said ingredients being infusible during the process of manufacture and another being softened by heat during manufacture sufficiently to bind the ingredients into a coherent mass.
- 60 9. The combination of a resistive conductor, and a solid insulating material embedding said conductor, said material composed of different ingredients one of which is fusible and another of which is infusible and having a coefficient of expansion higher than that of the conductor.
- 65 10. The combination of a resistive conductor, a support, and an insulating material embedding said conductor and adhesively engaging the support, said material containing as one ingredient an infusible substance having a coefficient of expansion higher than that of the conductor, and

containing another ingredient in the form of a vitreous material which serves to bind the parts together in the form of a solid coherent mass.

11. The combination of a resistive conductor, said conductor being in the form of a braid, and an insulating material embedding said conductor, one ingredient of said material having a coefficient of expansion higher than that of the conductor. 80

12. The combination of a resistive conductor, an insulating material embedding said conductor, said material being infusible, and an outer coating of vitreous material. 85

13. The combination of a resistive conductor, said conductor having a low temperature coefficient and a high coefficient of expansion, and an insulating material embedding said conductor, said material being infusible and containing an ingredient whose coefficient of expansion is higher than that of the conductor. 90

14. The combination of a resistive conductor, and an insulating material embedding said conductor, said material being formed of different ingredients, one of said ingredients having a coefficient of expansion higher than that of said conductor and the said coefficient of expansion being substantially unaffected by the heat of manufacture. 95

15. The combination of a support, a resistive conductor having a coefficient of expansion higher than that of the support, and a coating which attaches the conductor to the support, the coefficient of expansion of the coating being higher than that of the support and less than that of the resistive conductor. 100

16. The combination of a resistive conductor, and an insulating, protective, supporting, heat conducting, infusible material embedding said conductor, said coating being applied to the conductor in the form of a powder and formed by heat into a coating which is infusible and adhesive, said coating containing at least one ingredient whose coefficient of expansion is higher than that of said conductor. 105

17. The combination of a resistive conductor, and a protective insulating material embedding said conductor, said material being applied as a powder and formed by heat into a tough coherent layer of insulating material and which is subjected to a heat sufficient to cause the powdered material to cohere without causing the coating as a whole to fuse enough to flow or to obtain a glazed surface, said coating containing at least one ingredient whose coefficient of expansion is higher than that of said conductor. 110

18. The combination of a resistive conductor, and an insulating, infusible composition adherent thereto, said composition containing fluorspar or its equivalent. 115

19. The combination of a resistive conductor, and an insulating, infusible composition adherent thereto, said composition containing in its native state a mineral having a coefficient of expansion higher than that of the conductor and a binding material. 120

20. The combination of a support of insulating material, a resistive conductor, said conductor having a coefficient of expansion higher than that of said support, and a layer of insulating material applied in a finely divided state and forming a solid layer of material in which said conductor is embedded, the coefficient of expansion of said layer of material being between that of said conductor and that of said support. 125

21. The combination of a cylindrical support of insulating material, a resistive conductor, and a layer of insulating material applied in a finely divided state and forming a solid layer of material in which conductor is embedded, said layer of material having a coefficient of expansion between that of said support and that of said conductor. 130

22. The combination of a cylindrical support of insulating material, a resistive conductor, and a layer of insulating material upon said support and in which said conductor is embedded, said layer of insulating material containing an ingredient having a coefficient of expansion higher than that of said support and higher than that of said conductor. 135

In testimony whereof I affix my signature, in presence of two witnesses.

II. WARD LEONARD.

Witnesses:

L. K. SAGER,  
GEO. A. HOFFMAN.